

## UNITED STATES PATENT OFFICE.

TRYGVE D. YENSEN, OF SWISSVALE, PENNSYLVANIA, ASSIGNOR TO WESTINGHOUSE ELECTRIC & MANUFACTURING COMPANY, A CORPORATION OF PENNSYLVANIA.

## FORGEABLE ALLOY OF IRON AND NICKEL.

No Drawing.

Application filed April 18, 1919. Serial No. 290,922.

*To all whom it may concern:*

Be it known that I, TRYGVE D. YENSEN, a citizen of the United States, and a resident of Swissvale, in the county of Allegheny and State of Pennsylvania, have invented a new and useful Improvement in Forgeable Alloys of Iron and Nickel, of which the following is a specification.

My invention relates to alloys of iron and nickel and it has, for its object, the provision of alloys of this character which shall be readily forgeable over a wide range of temperatures.

It has been known for some time that pure alloys of iron and nickel do not forge readily at ordinary forging temperatures and it is necessary, in order to make them forgeable, to add small amounts of some alloying element. Manganese has been used for this purpose to such extent that it has come to be regarded as a necessary constituent of nickel steels.

I have now found that titanium can also be used to make iron-nickel alloys forgeable and that this element serves the purpose even more effectively than manganese. In practising my invention, a suitable proportion of titanium is combined with the iron and nickel forming the alloy in any manner desired, the proportion of titanium employed depending upon the relative proportions of nickel and iron in the alloy and, to some extent, upon impurities which may be present in the metals employed.

I have ascertained, however, that, by the addition of from 0.1 to 1% titanium, all iron-nickel alloys are rendered forgeable at all temperatures from black up to bright red heat, that is at temperatures ranging from below 500° to over 900° C.

While I do not wish to be restricted to any specific proportion of titanium in iron-nickel alloys, I have found that, for pure alloys containing from 0 to 50% nickel and the balance iron, the addition of titanium to an amount equal to 2% of nickel content may be made with satisfactory results and that, for alloys containing 50 to 100% nickel and the remainder iron, an addition of titanium to the amount of 2% of the iron content will

insure satisfactory results. In other words, the amount of titanium employed in any iron-nickel alloy may comprise substantially 2% of the content of the lesser metal.

I have found that iron-nickel alloys containing titanium are more readily forged at ordinary temperatures than corresponding alloys containing manganese and that this is particularly true if the titanium is present in substantially the proportions above specified. Of course, if manganese is present as an impurity, the amount of titanium added should be less, and it is possible that the presence of certain other impurities may also require a slight change in the proportion of titanium employed. For these reasons, I do not wish, in any way, to limit my invention but intend, in the appended claims, to cover it as broadly as the state of the art permits.

I claim as my invention:

1. A forgeable alloy comprising unequal quantities of iron and nickel and a relatively small amount of titanium, the amount of titanium varying in proportion to the amount of the lesser metal present.

2. A forgeable alloy comprising unequal quantities of iron and nickel and a small amount of titanium, the amount of titanium being substantially 2% of the amount of the lesser metal present.

3. A forgeable alloy comprising iron, a lesser amount of nickel and a relatively small amount of titanium, the amount of titanium varying in proportion to the amount of nickel present.

4. A forgeable alloy comprising iron, a lesser amount of nickel and titanium, the amount of the latter being substantially 2% of the amount of the nickel.

5. A forgeable alloy comprising iron and nickel and a small amount of titanium, the amount of titanium being substantially 2% of the amount of the lesser metal.

6. A forgeable alloy consisting of iron, nickel and titanium, the amount of titanium being between .1 and 1%.

In testimony whereof, I have hereunto subscribed my name this 3rd day of April, 1919.

TRYGVE D. YENSEN.